

# United States Patent [19]

Patterson

[11] 3,922,888

[45] Dec. 2, 1975

[54] **WARP KNIT TWILL, SHARKSKIN AND PIQUE FABRICS**

[75] Inventor: **Thomas E. Patterson, Pickens, S.C.**

[73] Assignee: **Deering Milliken Research Corporation, Spartanburg, S.C.**

[22] Filed: **Sept. 11, 1974**

[21] Appl. No.: **505,037**

[52] U.S. Cl. .... **66/192; 66/195**

[51] Int. Cl.<sup>2</sup> .... **D04B 21/00**

[58] Field of Search ..... 66/190, 192, 193, 194,  
66/195, 86 R

[56] **References Cited**

UNITED STATES PATENTS

|           |         |                 |          |
|-----------|---------|-----------------|----------|
| 2,012,355 | 8/1935  | Schonfeld ..... | 66/192 X |
| 2,149,031 | 2/1939  | Schonfeld ..... | 66/192 X |
| 2,149,032 | 2/1939  | Schonfeld ..... | 66/192 X |
| 2,153,645 | 4/1939  | Schonfeld ..... | 66/192   |
| 2,183,108 | 12/1939 | Schonfeld ..... | 66/192   |
| 3,109,302 | 4/1959  | Vitek .....     | 66/193   |
| 3,552,155 | 1/1971  | Hartung .....   | 66/192   |
| 3,733,859 | 5/1973  | Wittmann .....  | 66/193   |

FOREIGN PATENTS OR APPLICATIONS

|         |         |               |
|---------|---------|---------------|
| 324,028 | 5/1970  | Sweden        |
| 142,726 | 12/1961 | U.S.S.R.      |
| 33,601  | 11/1964 | Germany ..... |

OTHER PUBLICATIONS

Mayer Pattern No. 41/040, (1971).

Mayer Pattern No. 51/020, (1971).

Article No. TTIEI-4200/0403/03.

Mayer-Sample No. 4/4368a, (1970).

Article:TTI-W/E, 4201/202/181, (1971).

Article:TTI-W/E-WI, 4201/0202/171, (1971).

Article:TTI/E-WI, 4252/0411/01, (1968).

Mayet Sample No. 51/058, (1971).

Mayer Sample No. 41/180, (1971).

Paling, "Warp Knitting Technology," 2nd Ed., 1965, London, pp. 173-175, FIG. 134J.

*Primary Examiner*—Ronald Feldbaum  
*Attorney, Agent, or Firm*—H. William Petry; L. J. Wilburn, Jr.

[57] **ABSTRACT**

Warp knit twill, sharkskin or pique fabrics having a ground fabric structure formed by one or more yarns knit in every course and every wale to provide a ground structure, and yarns alternately laid into the ground structure in a pattern which advances course-wise as it alternates wale wise resulting in an effect which appears diagonally or obliquely to the course and wale directions throughout one or more surfaces of the fabric. Each of the laid-in yarns is substantially within a wale, and periodically makes an excursion toward or into an adjacent wale, laying in around the bases of two lap portions of yarn which terminate in that adjacent wale, the laid in yarn pulling the bases of those laps toward the wale in which the laid in yarn primarily lies, thereby periodically disrupting the uniformity of the technical back side of the warp knit fabric, and simultaneously tightening the loop which joins the two aforementioned laps thereby distorting the technical face of the warp knit fabric, to provide a pattern effect.

34 Claims, 21 Drawing Figures



FIG. 1B



FIG. 1

FIG. 2B



FIG. 2



FIG. 3B



FIG. 4B



FIG. 3



FIG. 4



FIG. 5B



FIG. 6B



FIG. 5



FIG. 6





FIG. 7



FIG. 8

FIG. 9







FIG. 12

FIG. 13



FIG. 14



FIG.15



## WARP KNIT TWILL, SHARKSKIN AND PIQUE FABRICS

This invention relates in general to simulated twill, sharkskin, and pique fabrics, and more specifically to warp knit twill, sharkskin, and pique fabrics, including warp knit elastic fabrics having the surface effects of twill, sharkskin, and pique fabrics.

Known twill, sharkskin, and pique fabrics, have typically been produced by weaving yarns to produce a pattern which extends obliquely to the warp and weft directions which characterize woven fabrics. More specifically, woven twills have the appearance of diagonal lines or ribs produced by passing the weft threads over one and under two or more warp threads, instead of merely passing under the next one warp thread. Woven piques have the appearance of raised diamond or hexagonal shaped patterns extending diagonally or obliquely to the warp and weft directions on the surface of the fabric. Woven sharkskins are like very fine piques having the appearance of an animal skin pattern, for example, a diamond-like pattern extending diagonally or obliquely to the warp and weft directions.

In contrast to woven fabrics, the structure of warp knit fabrics is more complicated. It is therefore not so easy to produce diagonal or oblique patterns in warp knit fabrics as it is in woven fabrics. However, warp knit fabrics have distinct advantages over woven fabrics, including the fact that warp knit fabrics are more extensible and therefore more readily accommodate the movements of a wearer of garments manufactured from warp knit fabrics. In addition, warp knit fabrics are today typically made of materials which are less prone to creasing and wrinkling, and the warp knit fabric structure itself provides improved resistance to creasing and wrinkling, thereby providing a fabric which is easier to care for than woven fabrics. Still further, warp knit fabrics have in the last few years been manufactured in quite elastic form, including highly elastic spandex yarns, for example, to provide light weight elastic fabrics, which when manufactured into garments readily conform to body curvatures and may even provide some support. Such fabrics have become particularly popular in applications such as swimsuits. However, such elastic fabrics are typically made having uniform, flat surfaces, with visual effects usually being provided by use of yarns of different color, or by fabric printing techniques.

Furthermore, while bare elastic yarns provide desirable high elastic elongations and stretch recovery, such yarns also have certain undesirable characteristics which typically must be dealt with in producing commercially acceptable elastic fabrics. One of those problems is that bare rubber and bare spandex yarns have an undesirably clammy feeling when brought into contact with human skin. Another undesirable characteristic is that bare rubber and bare spandex yarns are difficult to dye with dyes suitable for use in coloring commonly used textile yarns. Therefore if fabrics incorporating both the common yarns and the bare rubber or spandex yarns are to be dyed after being knit, it is desirable to cover the rubber or spandex yarns with the relatively inelastic yarns. Similarly, it is desirable to cover bare rubber or spandex yarns with the relatively inelastic yarns in order to avoid direct contact between the undesirably clammy rubber or spandex yarns and human skin when garments made from such fabrics are

worn next to the skin. There is a continuing need for warp knit elastic fabric structures wherein the desirable elasticity characteristics of bare rubber and spandex yarns may be used, while minimizing yarn consumption of both elastic and inelastic yarns per unit fabric area. There is also an apparent absence of elastic fabrics having twill, sharkskin and pique surface effect.

### BRIEF SUMMARY OF THE INVENTION

It is therefore an object of this invention to provide warp knit fabrics which overcome the above-noted disadvantages of prior art fabrics. It is more specifically an object of this invention to provide warp knit twill, sharkskin, and pique fabrics, and particularly warp knit elastic fabrics having twill, sharkskin, and pique surface effects.

The foregoing objects and others are accomplished in accordance with this invention by providing a ground structure formed by one or more hard or texturized, relatively inelastic yarns knit in every course and every wale to provide a rather opaque ground structure, and alternately laying yarns into that ground structure in a pattern which advances coursewise as it alternates wale wise to result in an effect which appears diagonally or obliquely to the course and wale directions throughout one or more surfaces of the resultant fabric. Each of the laid-in yarns is laid substantially within a wale, and periodically makes an excursion toward or into an adjacent wale, laying-in around the bases of two lap portions of yarn which terminate in that adjacent wale, the laid in yarn pulling those laps toward the wale in which the laid-in yarn primarily lies, thereby periodically disrupting the uniformity of the technical back side of the warp knit fabric, and simultaneously tightening the loop which joins the two aforementioned laps thereby distorting the technical face of the warp knit fabric, to thereby provide a pattern effect. The laid-in yarns may be of any desired type, including hard yarns, textured yarns, or even relatively highly elastic yarns.

### BRIEF DESCRIPTION OF THE DRAWINGS

For a better understanding of the invention as well as other objects and further features thereof, reference is made to the following detailed disclosures of preferred embodiments of the invention taken in conjunction with the accompanying drawings thereof, wherein:

FIG. 1 is an about 10 $\times$  photomicrograph of the technical face of a warp knit twill fabric of the present invention, and FIG. 1B is a photomicrograph of the technical back of the same fabric.

FIG. 2 is an about 10 $\times$  photomicrograph of the technical face of a warp knit sharkskin fabric of the present invention, and FIG. 2B is a photomicrograph of the technical back of the same fabric.

FIG. 3 is an about 10 $\times$  photomicrograph of the technical face of a warp knit sharkskin fabric of the present invention, and FIG. 3B is a photomicrograph of the technical back of the same fabric.

FIG. 4 is an about 10 $\times$  photomicrograph of the technical face of a pique fabric of the present invention, and FIG. 4B is a photomicrograph of the technical back of the same fabric.

FIG. 5 is an about 5 $\times$  photomicrograph of the technical face of a warp knit pique fabric of the present invention, and FIG. 5B is a photomicrograph of the technical back of the same fabric.

FIG. 6 is an about 5 $\times$  photomicrograph of the technical face of a warp knit pique fabric of the present in-

vention, and FIG. 6B is a photomicrograph of the technical back of the same fabric.

FIG. 7 is a point diagram schematically illustrating the patterns by which each of four yarn sets or warps are knit into a fabric of the present invention.

FIG. 8 is a point diagram schematically illustrating the patterns by which each of four yarn sets or warps are knit into another fabric of the present invention.

FIG. 9 is a point diagram schematically illustrating in superimposed form, the stitch pattern by which the four yarn sets of FIG. 8 are knit together to form a fabric according to the present invention.

FIG. 10 is an about 18 $\times$  scanning electron photomicrograph of the technical back of a fabric made according to the pattern illustrated in FIG. 9, said fabric being extended in both the course and wale directions.

FIG. 11 is an about 18 $\times$  scanning electron photomicrograph of the technical face of a fabric knit according to the pattern illustrated in FIG. 9, said fabric being extended in both the course and wale directions.

FIG. 12 is a point diagram schematically illustrating in superimposed form, the stitch patterns by which the four yarn sets of FIG. 7 are knit together to form a fabric according to the present invention.

FIG. 13 is a point diagram schematically illustrating in superimposed form, another stitch pattern by which the four yarn sets of FIG. 7 are knit together to form another fabric according to the present invention.

FIG. 14 is a point diagram schematically illustrating in superimposed form, another stitch pattern by which the four yarn sets of FIG. 8 are knit together to form another fabric according to the present invention.

FIG. 15 is a point diagram schematically illustrating in superimposed form still another stitch pattern by which the four yarn sets of FIG. 8 are knit together to form still another fabric according to the present invention.

#### DETAILED DESCRIPTION OF THE PREFERRED EMBODIMENTS

The warp knit twill, sharkskin, and pique fabrics of the present invention are made by knitting one or more yarns into a rather opaque ground structure, and alternately laying threads into that ground structure in patterns which sequentially or periodically distort the technical back and/or technical face of the fabric to provide an effect which appears diagonally or obliquely to the course and wale directions throughout one or both faces of the fabric. The ground structure is typically knit in every course and every wale, and is typically formed of one or more hard or textured, relatively inelastic yarns. The yarns which are laid into the ground structure are typically laid-in in a pattern which alternates walewise and which advances course-wise so that the surface effects which result from the laid-in yarn appear diagonally or obliquely to the course and wale directions.

One preferred way of making the warp knit twill and sharkskin fabrics of the present invention is to knit one or more types of yarns together using the stitch pattern

Bar 1: 2-0, 2-4

Bar 2: 2-4, 2-0

Bar 3: 4-4, 2-2, 4-4, 0-0

Bar 4: 4-4, 0-0, 4-4, 2-2

said stitch pattern being given in Raschel designations. Those skilled in the art will appreciate that such a stitch pattern, or combination of bar movement patterns, conventionally define the coordinated movements by

which the guide bars feed yarns to the knitting needles during knitting, and such a stitch pattern also defines the way in which the yarns lie in relationship to each other in the resultant fabric. Typically, two sets of 5 yarns, usually of the same type, are knit according to the Bar 1 and Bar 2 patterns, to form a substantially uniform ground fabric structure, which absent the sets of yarns laid-in by Bars 3 and 4, would not itself illustrate any extraordinary surface effect. Other yarns, 10 which may be the same type as the yarns used in the ground structure, or different, are laid-into the ground structure according to the Bar 3 and Bar 4 patterns. The foregoing patterns for Bars 1, 2, 3, and 4, are schematically illustrated in point diagram notation in FIG. 15 7.

In the present invention, the ground structure is typically formed of one or more yarn sets or warps which knit stitch loops in every course and every wale. In the stitch pattern illustrated in FIG. 7, the ground fabric is 20 formed from two warps or sets of yarns, one yarn of each of the two warps knitting in every course and every wale. In actual practice this would be done by fully threading Bar 1 and Bar 2 across the appropriate desired fabric width on a warp knitting machine, for example a tricot or a Raschel machine, and knitting those fully threaded bars, using the stitch pattern, or bar movement patterns, disclosed above and shown in FIG. 7. Such warp knitting machines are typically provided with appropriate pattern chains or cams to operate the 30 guide bars in accordance with a desired stitch pattern. While the ground structure is thus formed with two full warps of yarns, the yarns which are laid-in according to the Bar 3 and Bar 4 patterns illustrated in FIG. 7, are laid-in using two complementary warps, each threaded one-in, one-out, one of which is placed in the fabric by the Bar 3 pattern, and the other of which is placed in the fabric by the Bar 4 pattern. The total number of 35 ends of laid-in yarns may therefore be approximately equal to the total number of ends in one of the two full warps which are knit together by the patterns of Bar 1 and Bar 2 to form the ground fabric structure.

The most common way to alternate the respective 40 yarns of two complementary warps, as typically used for placing the inlaid Bar 3 and Bar 4 yarns in a fabric, is to prepare one warp for Bar 3, single ends of which are threaded one-in, one-out through alternate guides of a third bar of a warp knitting machine across the desired fabric width, and prepare another complementary warp from which single ends are threaded one-in, one-out, through alternate guides of a fourth guide bar of the warp knitting machine. However, there are other 45 ways of alternating the yarns of the two complementary warps to still place a full complement of inlaid yarns in the fabric while still achieving the desired surface effects of the present invention. For example, the yarns of each of Bar 3 and Bar 4 could be placed in the fabric by threading those bars on the machine two-in, two-out, respectively, or three-in, three-out, respectively. Furthermore, the Bar 3 and Bar 4 warps may be 50 differently threaded, but still complementary. For example, the warp fed to Bar 3 of the knitting machine may be threaded two-in, one-out, through the guides of the third guide bar across the desired fabric width, and the complementary fourth guide bar warp threaded two-out, one-in, through the guides of the fourth guide bar. While such variations in how the alternating laid-in 55 threads are placed in the fabric will make some variation in the resultant surface effects, for example they

may vary the angle at which the dominant lines of the pattern intersect the wale and course lines of the warp knit fabric, the principles by which the surface effects are created in such warp knit fabrics are basically the same. In further variations of the present invention, the total number of laid-in yarns need not comprise a full warp. In this way, ground fabrics having stripes of twill, sharkskin or pique surface effects throughout their length, may be produced.

Two of the aforementioned ways of alternating the laid-in yarns in fabrics using the stitch patterns illustrated in FIG. 7, are shown in FIGS. 12 and 13. In FIG. 12, the Bar 3 and Bar 4 yarns are alternated one-in, one-out, and in the FIG. 13 combination, the Bar 3 and Bar 4 yarns are alternated two-in, two-out. The results of making changes such as those illustrated by the combinations of FIGS. 12 and 13, may be visually appreciated by comparing FIGS. 1 and 2, which show fabrics which are made using the combination in FIG. 12, with the fabric of FIG. 3, which shows a fabric manufactured using the combination of FIG. 13. FIG. 1 shows a warp knit twill fabric of the present invention, and FIG. 2 shows a warp knit fabric of the present invention which is more akin to a sharkskin fabric, produced using the same yarns and stitch pattern used in making the fabric shown in FIG. 1; however, the length of yarn fed from one of the warps which forms the ground fabric was reduced, thereby altering the appearance of the surface effect. This illustrates another way in which the basic principles of the present invention may be used to create a somewhat different surface effect. FIG. 3 shows a fabric which exhibits an even more accentuated sharkskin effect produced by the stitch pattern illustrated in FIG. 13.

A preferred way of making the warp knit pique fabrics of the present invention is to knit one or more types of yarns together using the stitch pattern

Bar 1: 2-0, 2-4

Bar 2: 2-4, 2-0

Bar 3: 4-4, 2-2, 4-4, 2-2, 4-4, 2-2, 4-4, 0-0

Bar 4: 4-4, 2-2, 4-4, 0-0, 4-4, 2-2, 4-4, 2-2

said stitch pattern being given in Raschel designations. As in the previously described fabrics of the present invention, one or more yarns may be knit, usually in every course and every wale to form a ground fabric structure and in the fabric defined by this stitch pattern, or combination of bar movement patterns, two warps or sets of yarns are knit together, one by the pattern of Bar 1, and another by the pattern of Bar 2, to form a substantially uniform ground fabric structure. Again, two complementary partial warps of yarn are laid into the fabric by the patterns of Bar 3 and Bar 4, and it is the laid-in yarns which create surface effects in the resultant fabric. FIG. 8 schematically illustrates the foregoing pattern of Bars 1, 2, 3, and 4 in point diagram notation.

The points diagrams of FIG. 8 are also helpful in illustrating the present invention, in that it can be seen that the yarns which are laid into the structure by the patterns of Bar 3 and Bar 4 are generally laid into a single wale, for example the wales labelled A in FIG. 8, and those laid-in yarns only periodically make an excursion toward or into an adjacent wale labelled B in FIG. 8. Now that this principle has been pointed out in FIG. 8, it is also clear that yarns laid into fabrics in accordance with the patterns of Bar 3 and Bar 4 of FIG. 7, also lie primarily in one wale, labelled A' in FIG. 7, and periodically make an excursion toward or into the adjacent

wale labelled B' in FIG. 7. As previously mentioned, the alternating laid-in yarns appear to advance course-wide as they advance wale-wise to provide the surface effects of the present invention. The wale-wise alternation has previously been explained. The course-wise advance of the pattern of the alternate laid in yarns, may best be explained by following in successive wales the course-wise advance of those portions of the laid-in yarns which make an excursion out of the wale in which

10 a particular yarn is primarily laid-in, toward or into the adjacent wale. This is illustrated, for example, in FIG. 7 where it is seen that the Bar 4 yarn first makes an excursion into wale B' on course II', and then the Bar 3 yarn makes an excursion into its adjacent wale B' in course IV'. Returning then to Bar 4 yarn, it next makes an excursion into its adjacent wale B' in course VI', and then the Bar 3 yarn makes an excursion into its adjacent wale B' finally in course VIII'. It will be appreciated that when the yarns are laid-in according to the 15 patterns of FIG. 8, that the Bar 4 yarn first makes an excursion into adjacent wale B on course IV, while the Bar 3 yarn first makes an excursion into its adjacent wale B in course VIII.

A simple combination of the patterns of FIG. 8, is 20 shown in FIG. 9 where two full warps of yarns are schematically illustrated as being knitted according to each of the Bar 1 and Bar 2 patterns, respectively, and two complementary half warps, alternately threaded one-in, one-out, are schematically illustrated laid-into the aforesaid ground structure according to the Bar 3 and Bar 4 patterns. The patterns schematically illustrated in FIG. 9 illustrate even more fully the course-wise progression of the periodic excursions in the laid-in yarns, and why those combinations of laid-in yarns 25 produce diagonal or oblique surface effects in the fabrics of the present invention. For example, observe the excursions of the laid-in yarns as one moves from the yarns laid-into wale C to the yarn laid-into wale D to the yarn laid-into wale E, and eventually to the yarn laid-into wale F. Accompanying that wale wise progression, it is seen that the excursion in the laid-in yarns occurs in courses IV, VIII, XII, and XVI, respectively, and that those excursions of the laid-in yarns lie on a line X, which is oblique to both the wale and course directions 30 of the fabric.

The way in which the surface effects caused by the excursions of the laid-in yarns, is photomicrographically shown in FIGS. 10 and 11, which are respectively about 18 $\times$  scanning electron photomicrographs of the 35 technical back and technical face of a fabric made according to the pattern shown schematically in FIG. 9 the fabric having been photomicrographed when extended in both the course and wale directions.

Since the course-wise progression of the excursions 40 of the laid-in yarns is advanced the same number of courses between excursions in each of the two laid-in yarns, it does not matter at which side edge of the fabric one starts in locating such an oblique line on a diagram such as FIG. 9. For example, one can just as easily 45 locate such an oblique line by considering the excursions of the yarns which are primarily laid-in wales G, F, E, and D, respectively, which lie on a substantially straight line Y, which is likewise oblique to both the wale and course directions in the fabric of FIG. 9. However, so long as the number of courses between excursions in the two laid-in sets of yarns is the same, and as 50 long as the excursions occur on different courses in the 55 yarns of the two different laid-in warps, it does not matter

ter how many courses the individual excursions of the laid in yarns of one warp are offset from the excursions of the yarns of the other laid-in warp, since any such offsetting will produce the desired oblique surface effects in the fabrics of the present invention.

One way in which the excursions of the laid in yarns manifest themselves in the fabric of the present invention, is that in making an excursion toward or into the wale adjacent to the wale in which a laid in yarn primarily lies, the laid-in yarn loops or passes about the base of two lap portions of one of the ground fabric yarns, and tends to pull the bases of those lap portions, which otherwise extend in directions away from the excursion of their associated laid-in yarn, toward the wale in which that laid-in yarn primarily lies, giving the appearance that those two laps actually extend across approximately two wales. This is shown, for example, in FIG. 10 where the path of laid in yarns K, L, M, and N have been superimposed upon the photomicrograph, and at each of the excursions of these yarns, which tend to pull the base of laps which terminate in the adjacent wale back toward the wale in which the laid-in yarn primarily lies, those distended laps have been labelled 20. It is readily seen that those laps apparently terminate somewhere between the wale in which the laid-in yarn which is pulling those laps primarily lies, and the adjacent wales toward which the excursion of the laid in yarn took place. Using as a point of reference the point at which the bases of the distended laps seem to disappear between the wales, it can be seen that the effect caused by the excursions of the laid in yarns progresses wale-wise throughout the fabric along oblique lines represented by lines X' and Y'. Since point diagrams are usually drawn as if looking down upon the technical back of the fabric, the apparent paths of the laid-in 35

yarns shown in FIG. 9 and FIG. 10 are similar. FIG. 11 then shows the paths of the laid-in yarns superimposed upon a photomicrograph of the technical face of a fabric of the present invention, the same fabric whose technical back was shown in FIG. 10, and whose stitch pattern is shown in FIG. 9. The paths of the laid-in yarns have been labelled K', L' and M', substantially corresponding to the designations used in FIG. 10. Of course in this face view of the fabric, the excursions of the laid-in yarns take place toward the opposite edge of the fabric. In the face view of FIG. 11 the lap portions of one of the ground yarns, which are distended towards each of the wales in which the laid in yarns primarily lie, are visible, but that portion of those laps which extends behind a wale and away from the excursion of their associated laid-in yarn, have been superimposed on the photomicrograph of FIG. 11, and labelled with the numeral 20'. FIG. 11 also shows that the stitch loops 21, which connect the laps 20' which are distended on the technical back of the fabrics of the present invention, are distended on the technical face of the fabric so that each of the stitch loops 21 connecting correspondingly distended laps 20', is canted more obliquely to the wale line than the other loops in that wale line. These extraordinarily canted loops form a wale-wise progression on the face of the fabric, those canted loops lying on a line which is also oblique to both the wale and course directions of the fabrics of the present invention, as indicated by lines X'' and Y''. As thus shown on the face of the fabric in FIG. 11, and as shown on the technical back of the fabric in FIG. 10, it is clear that the advantageous twill, sharkskin, or pique patterns in the warp knit fabrics of the present invention

may occur on either the technical face or the technical back of the fabrics, and either side may be used as the desired effect surface, depending upon the application by the user.

Just as FIGS. 12 and 13 illustrated two combinations in which the pattern of FIG. 7 may be used in fabrics of the present invention, FIGS. 14 and 15, in addition to FIG. 9 illustrate various combinations in which the pattern of FIG. 8 may be used to produce fabrics according to the present invention. In FIG. 14, the yarns laid into the fabric according to the Bar 3 and Bar 4 patterns of FIG. 8, occur in a two-in, two-out alternation. The FIG. 15 pattern schematically illustrates a fabric wherein the laid-in yarns are placed in the fabric in alternation in three-in, three-out, sequences, respectively.

All of the foregoing makes it clear than the two sets of laid-in yarns of the present invention have stitch patterns wherein each laid-in yarn is primarily laid into one wale, and makes periodic excursions into an adjacent wale. The number of courses between the periodic excursions in each of the two sets of laid-in yarns is the same, but those excursions do not occur in the same course in both sets of laid-in yarns. The only further requirement to produce the advantageous twill, sharkskin, or pique effects of the present invention is that the length of the yarn laid-into each wale be short enough so that when the laid in yarn makes an excursion into or toward an adjacent wale, and when the fabric comes off the machine, the laps of the ground yarn around which the laid in yarn passed as it made the excursion into or toward the adjacent wale, are distended from their normal termination in the adjacent wale to an apparent termination closer to the wale in which the laid-in yarn primarily lies. It will also be appreciated that to effectively achieve these results, the excursions of the laid-in yarn should be coordinated with the ground fabric structure in such a way that the excursion or extended portion of the laid-in yarn passes around the base of laps which themselves otherwise extend in the opposite direction from the wale in which their associated laid-in yarn primarily lies.

Accompanying the distention of the pair of laps about which the laid-in yarn made the excursion, is the corresponding distortion or canting of the stitch loop which joins those two laps in the technical face of the fabric.

The types of yarns which may be used in the present invention may include any textile yarns capable of being knitted on a warp knitting machine a needle bar and a plurality of, usually at least three or four, guide bars. Since in the preferred fabrics of the present invention, the laid-in yarns, are almost entirely hidden or sandwiched within the wales of the fabrics, even yarns which have undesirable characteristics insofar as external appearance or effect is concerned, may be used as the laid-in yarn. For example, bare rubber or spandex elastic yarns have an undesirable clammy feeling when contacted by human skin, and typically give an undesirable "grin-through" in fabrics because such yarns are difficult to dye with dyes suitable for use in coloring more common textile yarns. But such yarns may be effectively covered when used as the laid-in yarns in the present invention. It is therefore clear that it is the ground fabric yarns which are exposed in the fabrics of the present invention, and which will provide those fabrics with desired esthetics such as hand and color. Similarly, it is the ground yarns, one of which is knit in every

course and every wale of the fabric, which will limit the extensibility of the fabrics of the present invention. But where relatively elastic yarns are used as the laid-in yarns, they provide good elastic elongation and stretch recovery to the inventive fabrics. In that regard it should be noted that a particularly preferred embodiment of the present invention is one wherein hard, or textured yarns are used in the ground fabric, and highly elastic yarns, such as spandex, are laid-into such a ground fabric. In such combinations, the present invention provides highly desirable elastic warp knit twill, sharkskin, or pique fabrics.

Accordingly, yarns suitable for use as the ground structure yarns in the present invention, include any of the well known relatively inelastic yarns, such as nylon, polyester, acetate rayon, or other yarns, in either rigid or textured form, and may include any natural yarns such as cotton or silk. Similarly, any of the foregoing yarns may be used as the laid-in yarns in the present invention. Furthermore, relatively elastic yarns such natural or synthetic rubber yarns, or any of the spandex yarns, such as DuPont's Lycra, may be laid-in to provide elastic warp knit fabrics according to the present invention. The relatively elastic yarn in the present invention is usually used in its bare condition, without covering such as a spiral winding. The word "yarn" is used herein in the generic sense to include any sort of elongate flexible member which may be knit on a warp knitting machine, and may include threads, filaments, strands, or yarns, whether they be monofilament, multi-filament, continuous filament, or comprise spun shorter fibers. It will of course be appreciated that the foregoing yarns are only representative of those useful in the present invention, and are in no way intended to limit the scope of application of the principles of the present invention.

During knitting of the fabrics of the present invention, the length of each set of yarns fed to the knitting machine (i.e., the runner length of each warp) need only be sufficient to accommodate the movements of the knitting elements of the machine without breaking yarn or breaking knitting elements. However, as mentioned earlier herein, the runner length of the laid-in yarns should be sufficiently short to cause the excursion portions of the laid-in yarns to pull the base of the laps of ground fabric yarn which the excursion loop around, out of their usual wale of termination and toward the wale in which the laid in yarn containing the excursion primarily lies, thereby also distending the 50 stitch loop which connects those laps. Any combination of runner lengths and resultant tensions which provides the desired result may be used. After the fabric is removed from the knitting machine, it may be dyed and finished by any means which the user may desire.

One of the primary advantages of fabrics of the present invention is that while the inlaid yarns are typically never pulled into a stitch loop or knitted into any course of the fabric, they are virtually never exposed on either surface of the cloth, so that they cannot be easily snagged, picked, or otherwise pulled out of the fabric. They therefore provide the warp knit surface effect fabrics of the present invention another advantage over woven fabrics, since the yarns which cause the desired twill, sharkskin, and pique surface effects in the warp knit fabrics of the present invention, cannot be snagged, picked pulled or run out of the fabric as is possible in the former woven fabrics.

10 The following examples are intended to illustrate various preferred embodiments of the present invention.

#### EXAMPLE I

5 A warp knit twill fabric is made by fully threading Bar 1 and Bar 2 of a Mayer 64 guage Raschel knitting machine with 1322 ends of 40 denier 13 filament DuPont Antron nylon and threading the third and fourth bars one-in, one-out, each with 661 ends of 140 denier Du-  
10 Pont T-127 Lycra spandex, and knitting those yarns together in the stitch pattern: Bar 1: 2-0, 2-4; Bar 2: 2-4, 2-0; Bar 3: 4-4, 2-2, 4-4, 0-0; and Bar 4: 4-4, 0-0, 4-4, 2-2. The Bar 1 runner length is about 55 inches per rack; Bar 2 runner length about 51 inches per rack; and  
15 Bars 3 and 4 each have runner lengths of about 5½ inches per rack; the Lycra yarns being extended about 104 percent as warped on the beam. The fabric is knit at about 60 stitches per inch on the machine. The resultant fabric is an opaque, warp knit elastic twill fabric  
20 having a twill surface effect as shown in FIGS. 1 and 1B, wherein the relatively elastic yarns are substantially covered by the ground yarns. In this fabric, as in the other fabrics of the present invention, either the technical back side, or the technical face side of the fabric  
25 may be used as the desired exterior effect surface.

While the greige fabric embodies the present invention, after knitting the fabric may be finished by any desired technique, specific finishing techniques not being a part of the claimed invention. For example, the greige 30 fabric taken from the knitting machine may then be run into a scray to relax the dry fabric. The fabric may then be removed from the scray and run through a wash box containing water at about 200°F with a small amount of detergent therein. The tension settings are set to run the fabric through the wash box in a relaxed condition. The fabric may be taken from the wash box and framed on a small tenterette, with overfeeds and tension controls set to wind the fabric onto a Burlington beam in a relaxed condition. The fabric may be Burlington beam  
35 machine dyed under atmospheric pressure, by steps which may include chemically scouring, rinsing, dying, heat fixation of the dye, and further rinsing. The fabric may then be extracted on a beam extractor, and heat set at a desired wale and course count.

#### EXAMPLE II

A warp knit sharkskin fabric is produced using a machine set up as described in Example I, except that in producing this fabric the Bar 2 runner length is about 48½ inches per rack. The resultant fabric is a warp knit elastic sharkskin fabric having surface effects as shown in FIGS. 2 and 2B.

#### EXAMPLE III

55 A warp knit sharkskin fabric is produced using a setup quite similar to that described in Example I, except that the Bar 2 runner length is about 51½ inches per rack, and instead of being threaded one-in, one-out, in each of Bars 3 and 4, the Lycra yarns are 60 threaded two-in, two-out, in each of guide bars 3 and 4. The resultant fabric is a warp knit elastic sharkskin fabric having the surface effects shown in FIG. 3 and 3B.

#### EXAMPLE IV

65 A warp knit pique fabric is produced by fully threading the first and second bars of a Mayer 64 guage Raschel knitting machine with 1322 ends of 40 denier 13 filament R-25 DuPont Antron nylon. Bars 3 and 4

were each threaded one-in, one-out, with 661 ends of 140 denier DuPont T-127 Lycra spandex yarns. These yarns were knit according to the stitch pattern: Bar 1: 2-0, 2-4, Bar 2: 2-4, 2-0, Bar 3: 4-4, 2-2, 4-4, 2-2, 4-4, 0-0; and Bar 4: 4-4, 2-2, 4-4, 0-0, 4-4, 2-2, 4-4, 2-2. The runner length of Bar 1 is about 52½ inches per rack; Bar 2 about 44 inches per rack; and Bars 3 and 4 each about 6.2 inches per rack, the Lycra yarns being extended about 104 percent as warped on the beam. The fabric was knit at about 80 stitches per inch on the machine. The resultant fabric is a warp knit elastic pique fabric having the surface effects shown in FIG. 4 and 4B, and the knit structure of the fabric is shown in more detail in FIGS. 10 and 11.

## EXAMPLE V

A warp knit pique fabric is produced using a machine setup as described in Example IV, except that the Lycra yarns in Bars 3 and 4 instead of being threaded one-in, one-out, are threaded two-in, two-out, in each of Bars 3 and 4. The resultant fabric is a warp knit elastic pique fabric having surface effects shown in FIG. 5 and 5B.

## EXAMPLE VI

A warp knit pique fabric is produced using a machine setup as described in Example IV, except that the Lycra yarns in Bars 3 and 4 instead of being threaded one-in, one-out, are threaded three-in, three-out, in each of Bars 3 and 4. The resultant fabric is a warp knit elastic pique fabric having surface effects as shown in FIG. 6 and 6B.

Although specific components, proportions, and arrangements of elements have been stated in the above description of preferred embodiments of this invention, other equivalent components and arrangements of elements may be used with satisfactory results and various degrees of quality, or other modifications may be made herein to enhance the invention to thereby increase its utility. For example, the ground fabric may comprise a single bar fabric, or may be knit using open stitch loops in any or all courses and wales. Also, the patterns stated herein have been given in Raschel designations, but those skilled in the art can readily translate those patterns into tricot designations. It will be understood that such changes of details, materials, arrangements of parts, and uses of the invention described and illustrated herein, are intended to be included within the principles and scope of the claimed invention. Any greige or finished fabric meeting the limitations of the appended claims is intended to be within the scope of the present invention.

What is claimed is:

1. A warp knit fabric comprising a first set of yarns forming a knit ground structure containing stitch loops in every course and wale, and second and third sets of yarns laid into the ground structure; each respective yarns of said second set primarily lying in one respective wale of the ground structure and periodically extending toward an adjacent wale, passing around at least two lap portions of one of the yarns of the ground structure, which lap portions otherwise extend in directions away from the portion of the yarn of the second set which extends toward the adjacent wale, and displacing those laps toward the wale in which the yarn of said second set is primarily lying; each respective yarn of said third set primarily lying in a respective wale of the ground structure and periodically extending toward

an adjacent wale, passing around at least two lap portions of one of the yarns of the ground structure, which lap portions otherwise extend in directions away from the portion of the yarn of the third set which extends toward the adjacent wale, and displacing those laps toward the wale in which the yarn of said third set is primarily lying; the yarns of the second and third sets making all their periodic extensions in the same direction, but with the yarns of the third set making their periodic extensions in different courses from the courses in which the yarns of the second set make their periodic extensions; said second and third sets of yarns being substantially covered by the yarns of the ground structure, and said fabric having a surface effect on at least one face thereof which appears to extend along line oblique to the course and wale directions in the fabric.

2. The warp knit fabric of claim 1, wherein the stitch loops of yarn on the technical face of the fabric which join the two laps which are displaced by each of the extending portions of the laid-in yarns, are more oblique with respect to the directions of the wales than the other stitch loops which comprise said wales.

3. The warp knit fabric of claim 1, wherein the yarns of said second set are primarily laid into different wales from the wales in which the yarns of said third set are primarily laid-in.

4. The warp knit fabric of claim 2, wherein a surface effect which appears to extend generally along lines oblique to the course and wale directions in said fabric appears on both faces of the fabric.

5. The warp knit fabric of claim 1, wherein the yarns of said second and third sets alternate across the course-wise width of the fabric in such a way that at least one yarn of said second set alternates across the width of the fabric with at least one yarn of said third set.

6. The warp knit fabric of claim 1, wherein the yarns of said second and third sets alternate across the course-wise width of the fabric in such a way that more than one yarn of said second set alternates across the width of the fabric with more than one yarn of said third set.

7. The warp knit fabric of claim 1, wherein the ground structure additionally comprises another set of yarns, which knit in every course on every wale in said ground structure.

8. The warp knit fabric of claim 1, wherein the laid-in yarns of said second and third sets comprise relatively elastic yarns, and said fabric is elastic.

9. The warp knit fabric of claim 8, wherein said relatively elastic yarns comprise spandex yarns.

10. The warp knit fabric of claim 7, wherein in said ground structure comprises said first set of yarns knit in the fabric in the pattern: 2-0, 2-4, and said another set of yarns knit in the fabric in the pattern: 2-4, 2-0, said patterns being given in Raschel designations.

11. The warp knit fabric of claim 6, wherein the yarns of said second set of yarns are laid-into the fabric in the pattern: 4-4, 2-2, 4-4, 0-0, and the yarns of said third set are laid-into the fabric in the pattern: 4-4, 0-0, 4-4, 2-2, said patterns being given in Raschel designations.

12. The warp knit fabric of claim 6, wherein the yarns of said second set of yarns are laid-into the fabric in the pattern: 4-4, 2-2, 4-4, 2-2, 4-4, 2-2, 4-4, 0-0, and the yarns of said third set are laid-into the fabric in the pattern: 4-4, 2-2, 4-4, 0-0, 4-4, 2-2, 4-4, 2-2, said patterns being given in Raschel designations.

13. The warp knit fabric of claim 10, wherein the 5  
yarns of said second and third sets alternate across the  
coursewise width of the fabric in such a way that at  
least one yarn of said second set alternates across the  
width of the fabric with at least one yarn of said third  
set, and the yarns of said second set of yarns are laid  
into the fabric in the pattern: 4-4, 2-2, 4-4, 0-0, and the  
yarns of said third set are laid-into the fabric in the pattern:  
10 4-4, 0-0, 4-4, 2-2, said patterns being given in  
Raschel designations.

14. The warp knit fabric of claim 10, wherein the  
yarns of said second and third sets alternate across the  
coursewise width of the fabric in such a way that at  
least one yarn of said second set alternates across the  
width of the fabric with at least one yarn of said third  
set, and the yarns of said second set of yarns are laid  
into the fabric in the pattern: 4-4, 2-2, 4-4, 2-2, 4-4,  
15 2-2, 4-4, 0-0, and the yarns of said third set are laid-into  
the fabric in the pattern 4-4, 2-2, 4-4, 0-0, 4-4, 2-2, 4-4,  
20 2-2, said patterns being given in Raschel designations.

15. A method of manufacturing a warp knitted fabric, comprising the steps of:

1. fully threading a front guide bar of a warp knitting  
machine across an approximate desired fabric  
width with a first plurality of yarns;

2. fully threading a second guide bar of said warp  
knitting machine across said approximate desired  
fabric width with a second plurality of yarns;

3. partially threading a third guide bar of said warp  
knitting machine alternately across said approximate  
desired fabric width with a third plurality of  
yarns;

4. partially threading a fourth guide bar of said warp  
knitting machine across said approximate desired  
fabric width alternately in an arrangement comple-  
mentary to the arrangement of yarns threaded  
through said third guide bar; and

5. operating said warp knitting machine, said guide  
bars feeding yarns to the needle bar of said ma-  
chine according to the combination of bar move-  
ment patterns:

front bar: 2-0, 2-4

second bar: 2-4, 2-0

third bar: 4-4, 2-2, 4-4, 0-0

fourth bar: 4-4, 0-0, 4-4, 2-2

45 said patterns being given in Raschel designations.

16. The method of claim 15, wherein said third and  
fourth guide bars are threaded with yarns comprising  
50 bare relatively elastic yarns.

17. The method of claim 15, wherein each yarn of  
said third and fourth pluralities is laid-into primarily  
one wale of the resultant fabric, and the length of each  
of said third and fourth pluralities of yarns fed to the  
needle bar is sufficiently short so that as the fabric is  
manufactured portions of each one of said yarns of said  
third and fourth pluralities extend toward a wale adja-  
cent to the wale in which said one yarn primarily lies,  
each said portion passing around two lap portions of a  
55 yarn from said first plurality of yarns, displacing those  
lap portions toward the wale in which said one yarn pri-  
marily lies.

18. A method of manufacturing a warp knitted fab-  
ric, comprising the steps of:

1. fully threading a front guide bar of a warp knitting  
machine across an approximate desired fabric  
width with a first plurality of yarns;

14  
2. fully threading a second guide bar of said warp  
knitting machine across said approximate desired  
fabric width with a second plurality of yarns;

3. partially threading a third guide bar of said warp  
knitting machine alternately across said approxi-  
mate desired fabric width with a third plurality of  
yarns;

4. partially threading a fourth guide bar of said warp  
knitting machine across said approximate desired  
fabric width alternately in an arrangement comple-  
mentary to the arrangement of yarns threaded  
through said third guide bar; and

5. operating said warp knitting machine, said guide  
bars feeding yarns to the needle bar of said ma-  
chine according to the combination of bar move-  
ment patterns:

front bar: 2-0, 2-4

second bar: 2-4, 2-0

third bar: 4-4, 2-2, 4-4, 2-2, 4-4, 2-2, 4-4, 0-0,

fourth bar: 4-4, 2-2, 4-4, 0-0, 4-4, 2-2, 4-4, 2-2,  
said patterns being given in Raschel designations.

19. The method of claim 18, wherein said third and  
fourth guide bars are threaded with yarns comprising  
bare relatively elastic yarns.

20. The method of claim 19, wherein each yarn of  
said third and fourth pluralities is laid-into primarily  
one wale of the resultant fabric, and the length of each  
of said third and fourth pluralities of yarns fed to the  
needle bar is sufficiently short so that as the fabric is  
manufactured portions of each one of said yarns of said  
third and fourth pluralities extend toward a wale adja-  
cent to the wale in which said one yarn primarily lies,  
each said portion passing around two lap portions of a  
30 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9

15

yarns, and said bare, relatively elastic yarns are substantially covered by the yarns of said first set.

24. The method of claim 22, wherein said second and third sets of yarns comprise bare, relatively elastic yarns, and said bare, relatively elastic yarns are substantially covered by the yarns of said first set.

25. The method of claim 23, wherein said relatively elastic yarns are elastically elongated before being laid into the ground fabric construction.

26. The method of claim 22, wherein the fabric is knitted on a warp knitting machine, and said first set of yarns is supplied to the knitting needles of said machine through a front guide bar fully threaded across an approximate desired fabric width, said another set of yarns is supplied to said knitting needles through a second guide bar fully threaded across said approximate fabric width, said second set of yarns is supplied to said knitting needles through a third guide bar partially and alternately threaded across said approximate fabric width, said third set of yarns is supplied to said knitting needles through a fourth guide bar partially and alternately threaded in an arrangement complementary to the arrangement of yarns threaded through said third guide bar, and operating said machine so that the front and second guide bars feed yarns to the needles according to the bar movement patterns:

front bar: 2-0, 2-4

second bar: 2-4, 2-0

said patterns being given in Raschel designations.

27. The method of claim 26, additionally comprising operating said third and fourth guide bars to feed yarns to the needles, in synchronization with the bar move-

16

ment patterns of said front and second bars, according to the bar movement patterns:

third bar: 4-4, 2-2, 4-4, 0-0

fourth bar: 4-4, 0-0, 4-4, 2-2

said patterns being given in Raschel designations.

28. The method of claim 26, additionally comprising operating said third and fourth guide bars to feed yarns to the needles, in synchronization with the bar movement patterns of said front and second bars, according to the bar movement patterns:

third bar: 4-4, 2-2, 4-4, 2-2, 4-4, 2-2, 4-4, 0-0

fourth bar: 4-4, 2-2, 4-4, 0-0, 4-4, 2-2, 4-4, 2-2

said patterns being given in Raschel designations.

29. The method of claim 26, wherein the arrangements in which said second and third sets of yarns are threaded through said third and fourth guide bars, respectively, is such that at least one yarn of said second set alternates with at least one yarn of said third set across said approximate fabric width as said second and third sets are laid into the ground construction.

30. The method of claim 29, wherein said second and said third sets of yarns comprise bare, relatively elastic yarns.

31. The method of claim 30, wherein said relatively elastic yarns are elastically elongated before being supplied through a guide bar.

32. The method of claim 21, wherein only one yarn is laid into each wale of the fabric.

33. The method of claim 26, wherein only one yarn is laid into each wale of the fabric.

34. The warp knit fabric of claim 1, wherein only one of the yarns laid into the fabric lies in each wale of the fabric.

\* \* \* \* \*

35

40

45

50

55

60

65

UNITED STATES PATENT OFFICE  
CERTIFICATE OF CORRECTION

Patent No. 3,922,888 Dated December 2, 1975

Inventor(s) Thomas E. Patterson

It is certified that error appears in the above-identified patent and that said Letters Patent are hereby corrected as shown below:

Column 1, line 11, the word "yarsn" should read --yarns--.

Column 2, line 7, the word "effect" should read --effects--.

Column 3, line 26, the word "is" should read --in--.

Column 6, line 32, the word "illustrated" which appears after "FIG. 9" should read --illustrate--.

Column 8, line 17, the word "than" should read --that--.

Column 8, line 50, after "machine", insert --having--.

Column 11, line 58, the word "yarns" should read --yarn--.

Column 12, line 45, the word "is" should read --in--.

Signed and Sealed this

Ninth Day of November 1976

[SEAL]

Attest:

RUTH C. MASON  
Attesting Officer

C. MARSHALL DANN  
Commissioner of Patents and Trademarks